

## UNITED STATES PATENT OFFICE.

GILBERT MICHEL, OF BAGNEUX, FRANCE, ASSIGNOR TO HART O. BERG, OF PARIS, FRANCE.

## PURIFICATION OF MAGNESIUM AND ITS ALLOYS.

No Drawing. Application filed February 5, 1925, Serial No. 7,156, and in France October 4, 1924.

Crude magnesium obtained either as recovery from waste or from the vessels in electrolytic manufacture, contains in almost all cases numerous impurities and especially 5 oxides and oxychlorides dispersed in the mass in the state of grains or granules. It is particularly difficult to wholly remove the oxides. In certain former processes the purification of the magnesium was attempted by 10 causing magnesium chloride to act upon the molten metal bath, assisted by an energetic stirring. In the case where the chloride of magnesium was added in excess there was added thickening bodies such as fluorides of 15 calcium or aluminum and other bodies the purpose of which was to form complexes with the chloride in excess.

But processes of this sort present the inconvenience that it is practically impossible 20 to know in advance the quantity of chloride necessary to saturate the impurities and furthermore there always remains in the bath, in spite of all precautions, traces of 25 chlorides or oxychlorides which is very harmful to the metal. Even if magnesium chloride and magnesium fluoride are added together, satisfactory results would not be secured.

The present invention has for its object a 30 process in which the impurities instead of being eliminated by the addition of a chloride acting as a principal purifying agent, are eliminated by the addition of magnesium fluoride without magnesium chloride. The fluoride in this case does not act to saturate 35 magnesium chloride which only exists in traces in the bath since no additional quantities are added during the process, but it acts as a principal purifying agent for the impurities and principally of the oxides contained in the mass.

Attempts have also been made to overcome 40 this difficulty by lowering the melting point of the magnesium or its alloys to the minimum by the addition of zinc, but it is found 45 that zinc can be alloyed with magnesium only with great difficulty and furthermore magnesium alloyed with zinc is found to deteriorate in the course of time. The metal or alloy which is thus obtained is of an unstable character and loses its useful qualities and mechanical properties after a time. It has been observed that the above mentioned alloy is 50 the less adapted for forging, rolling and the like thermo-mechanical operations employed 55 in metal working, according as the propor-

tion of zinc is larger. It is also found that such metals and alloys are not adapted for autogenous welding.

It is a known fact that magnesium or its alloys which are produced by the known 60 methods always contain traces of chlorides and oxychlorides, these being prejudicial to the good quality of the metal.

An object of the invention is the manufacture of metals or alloys having magnesium 65 as a base, which are perfectly stable and will not deteriorate with age or change their characteristic properties. The products of the invention are therefore particularly adapted to all the thermo-mechanical operations 70 employed in metal working, such as forging, rolling and the like, and which according to their composition possess qualities of hardness, elasticity, ductility and the like of a particularly valuable kind, these products being 75 also capable of autogenous welding.

The two essential features of the metals and alloys having magnesium as a base, the object of the present invention, consist in the 80 fact that they contain calcium, and that they are freed from all chlorides and oxychlorides by an adequate treatment.

Calcium has the property of lowering the melting point of magnesium in the same manner as zinc, which latter has been hitherto employed for this purpose, and by its use I am enabled to proceed with the operations of melting, refining and purifying under favorable conditions, avoiding all spontaneous ignition and excessive oxidation. The presence 90 of calcium in small quantities in the magnesium does not affect its useful properties, but on the contrary alloys are obtained which are of extreme lightness combined with great hardness. The proportions which are found 95 to produce the best results are 0.05% up to 0.3% of Ca. Magnesium containing calcium and magnesium alloys containing containing calcium have been found to be very well adapted for autogenous welding.

Due to the elimination of all impurities containing chlorine such as the chlorides and oxychlorides, for instance by the process to be hereinafter described, the said metals and alloys are particularly well adapted for forging, rolling and the like, and the good preservation of the metal is insured.

A method according to the invention of manufacturing the metal and its alloys is as follows:

- The melting point of the metal or alloy having magnesium as a base which is employed as the raw material is lowered by the addition of calcium and of a suitable flux; 5 the chlorides and oxychlorides are eliminated by stirring the mass in the presence of a chemical agent which may be so chosen as to simultaneously act as a flux; the surface of the metal is protected against oxidation by 10 the use of a layer of a reducing agent which also effects the reduction of all oxide impurities on the surface of the metallic bath.

I prefer to place the magnesium metal or alloy serving as the raw material in a crucible which is preliminarily sprinkled with magnesium fluoride  $MgF_2$ ; this latter substance will be further distributed among the pieces of metal and also spread upon the surface of the metallic mass. As soon as the 15 metal commences to melt, the mass is vigorously stirred in order to form an intimate mixture of the said metal and the magnesium fluoride. This latter acts both as a flux and as a purifier. It imparts fluidity to the magnesium or its alloys, and eliminates the chlorides and oxychlorides which rise to the surface of the bath.

When the metallic mass has become sufficiently fluid, I incorporate therein the 20 amount of the calcium which is desired according to the required properties of the metal; I prefer to add the calcium in the form of very small particles, for this state conduces to the rapid diffusion of the calcium throughout the magnesium, and the reaction even 25 takes place with such violence that a vigorous stirring of the mass results, this being most favorable for the intimate contact of the various constituents.

30 The small pieces of calcium can be for instance placed in a thin magnesium tube and the latter introduced into the center of the mass; the tube is soon melted, and the calcium at once dissolves in the bath, which 35 boils up to a considerable degree.

The surface of the metal bath is then 40 sprinkled with a reducing agent such as ammonium chloride  $NH_4Cl$ , which forms a crust on the surface and thus protects the metal 45 bath against the oxygen of the air and prevents all excessive oxidation of the same; at the same time the ammonium chloride re-

duces the oxides and oxychlorides which may have been formed or which have risen to the surface. In this manner, and without any 55 ignition or excessive oxidation, a metal or alloy having magnesium as a base is produced, which contains no zinc but contains calcium, and is freed from its prejudicial impurities and chiefly the chlorides and oxychlorides. 60

When magnesium of a moderate grade of purity is employed as raw material, I prefer to adopt the following proportions of the chemical agents before mentioned: 65

For 30 kg. of magnesium 30 to 40 grammes of magnesium fluoride and 30 to 60 grammes of ammonium chloride.

These quantities can be doubled or even tripled specially for the magnesium fluoride, 70 if the raw magnesium contains a great deal of impurities. In the appended claims, the expression "metallic magnesium material" is intended to cover magnesium itself, as well as alloys of magnesium. 75

I claim:

1. The process of purification of magnesium or its alloys which comprises forming complexes with the oxychlorides and oxides found in the bath by mixing same with magnesium fluoride acting as a main purifier, without adding a chloride, and collecting the complexes at the surface of the bath. 80

2. Process according to claim 1, consisting in producing the agitation of the bath by the 85 addition of calcium in a finely divided condition.

3. Process according to claim 1 consisting in producing the agitation by the addition of finely divided calcium enclosed in a cartridge of magnesium. 90

4. Process according to claim 1 consisting in also adding to the bath ammonium chloride to produce a reducing layer on the surface of the bath. 95

5. Process for purification of magnesium or its alloys consisting in adding magnesium fluoride to the bath, then incorporating finely divided calcium into the mass, and placing a layer of ammonium chloride on the surface 100 of the bath.

In testimony whereof I have signed my name to this specification.

GILBERT MICHEL.